

# UNITED STATES PATENT OFFICE.

JOSEPH EMILE GERNEILLE-DANLOY, OF MOULINS, FRANCE.

## COATING FOR MOLDS AND CORES.

1,218,394.

Specification of Letters Patent.

Patented Mar. 6, 1917.

No Drawing.

Application filed December 10, 1914. Serial No. 876,479.

*To all whom it may concern:*

Be it known that I, JOSEPH EMILE GERNEILLE-DANLOY, a citizen of the French Republic, residing at Moulins, Allier, in France, have invented certain new and useful Improvements in Coatings for Molds and Cores, of which the following is a specification.

The present invention relates to a product destined to replace black lead and other products usually employed to coat molds and cores made out of sand, which are intended to be dried or baked before casting.

This product can be employed for castings of steel, cast-iron, copper, bronze, aluminum and all metals in general.

My improved product is composed of coke dust, wood charcoal, pipe clay, and starch, the latter partly in the form of powdered raw starch and partly in the form of a dried starch paste.

Under the term "coke dust" I desire to be understood the impalpable powder derived from hard washed coke of a quality suitable for metallurgical operations broken and ground to a fine powder.

The ingredients named form a composition which when mixed with water to form a paste capable of being applied to the mold or core by means of a brush, produces a thin but hard and smooth coating which does not detract from the quality and appearance of the cast metal, prevents the adherence thereto of sand from the mold or core so that the castings do not need any subsequent cleaning, and enables castings to be obtained which are free from surface cracks and blemishes.

The resistant and protective qualities of coke dust and fire clay are already known in connection with coatings for molds and cores and flour has also been employed therewith in compositions for the same purpose. These compositions have hitherto been used without any special agglutinative additions, or in some instances sour beer has been proposed as an agglutinative. I have however found that the addition of dried

flour paste, which is in effect dextrin and is soluble in water (whereas flour itself is not fully soluble and only very slightly agglutinative) provides a perfect agglutinative and produces in combination with the other ingredients mentioned a composition the employment of which gives greatly improved results. The foregoing materials are employed in the new product in the following proportions:

|                        |       |    |
|------------------------|-------|----|
| Coke, washed           | 40 %  | 60 |
| Charcoal               | 32.5% |    |
| Pipe-clay              | 22.5% |    |
| Starch paste, dry      | 2 %   |    |
| Starch, raw, in powder | 3 %   |    |

These quantities may vary slightly according to the quality of the materials employed. These are pulverized together and very finely bolted, giving an impalpable and very homogeneous powder of a blackish shade.

This product is employed mixed with an equal volume of water, and is applied to the surface by means of a brush and when dried appears like an enamel varnish. The taking out of the sand is made without necessitating other work than the ordinary removal of the mold, obviating the rasping of the pieces after the casting. The castings obtained have a very smooth surface and the metals keep their qualities and their natural shade; the castings are very clean and do not soil when they are touched as do those obtained with the use of black lead or all other similar materials, which has a certain importance when the pieces have to be finished.

Moreover, the weight of the new product is 40% less than that of an equal quantity of black lead of good quality, which permits of a great economy from its use.

Having thus described my invention and the manner to work it out, I claim patent for:

1. A composition for use in coating sand molds and cores, comprising in combination coke dust, charcoal, pipe clay and raw

starch, together with dry starch paste to serve as an agglutinant substantially in the proportions herein set forth.

2. A composition for use in coating sand molds and cores comprising known carbonaceous mixtures previously employed for this purpose together with an agglutinant consisting of dry starch paste.

In witness whereof I have signed this specification in the presence of two witnesses.

JOSEPH EMILE GERNEILLE-DANLOY.

Witnesses:

JEAN GERMAIN,  
LOUIS GONICHON.